

**1**

2,713,539

**MANUFACTURE OF HIGH WET STRENGTH  
PAPER**

William F. Fowler, Jr., Donald R. Spear, and Lee K. Tong, Rochester, N. Y., assignors to Eastman Kodak Company, Rochester, N. Y., a corporation of New Jersey

No Drawing. Application February 14, 1951,  
Serial No. 210,986

8 Claims. (Cl. 92—3)

This application relates to the manufacture of a high wet strength sized paper obtained by beater sizing the pulp from which the paper is obtained with a polyalkyl acrylate and a wax dispersion.

Ordinarily, paper is sized to resist the penetration of liquids therein and to give the paper a certain amount of body. Also for many purposes it is desirable that the paper have a substantial wet strength, particularly where the paper is to come in contact with water or aqueous solutions of various types. The sizing of paper at the present time in many cases involves the precipitation in the pulp in a dispersed condition of stearic acid (or its aluminum salts) from a solution of sodium stearate by the addition of aluminum sulfate or the like thereto. Recently aluminum chloride has been suggested for this purpose.

To impart high wet strength to paper, the addition to the pulp dispersion of water soluble urea-formaldehyde resins or melamine-formaldehyde resins after the Jordaning operation, but prior to its dispersing on the wire of the paper machine, has been suggested. Although this method of preparing high wet strength paper has been found to be satisfactory in some instances, in other instances the presence of the formaldehyde resins has been considered objectionable, particularly where the prevalence of even a trace of formaldehyde cannot be tolerated. Also, the preparation of sized high wet strength papers in this fashion has involved several operations and a large quantity of expensive equipment.

Other methods of increasing the wet strength of paper have been proposed. For instance, latices of various types have been suggested as being suitable for this purpose. Many of these materials have been found to be unstable in the presence of ultraviolet light and also some of these materials contain sulfur, which is undesirable in some cases. Hydrosols of polyvinyl acetate have been suggested both as coating compositions for paper and for use in paper tub sizing operations. This resin, however, is not sufficiently hydrophobic to be useful as a sizing agent.

One object of our invention is to provide a method for use in the preparation of paper which simultaneously sizes the paper and increases its wet strength. Another object of our invention is to prepare a high wet strength paper, the dry strength of which is commensurate with that ordinarily obtained in paper manufacture. A further object of our invention is to provide a method of preparing high wet strength sized paper in which polyalkyl acrylate resins are employed in the pulp from which the paper is prepared.

We have found that by adding to a paper pulp while in suspension a polyalkyl acrylate and a wax dispersion, together with an acidic compound of aluminum, that the resulting paper obtained therefrom has both high wet strength and sized characteristics. We have found, however, that in order to obtain such a paper it is necessary to first provide the cellulose fibers with surfaces to

**2**

which both the polyalkyl acrylate and the wax dispersion will adhere.

The material which is added to the pulp suspension to render the cellulose fibers adherent of the sizing material is known as a "sizing aid" and may be either gelatin, the water soluble salt of 1-pimamic acid-maleic anhydride adduct, or the water soluble salts of abietic acid or of hydrogenated abietic acid. This sizing aid in aqueous solution is added to the pulp suspension preliminary to the addition of the sizing material as referred to herein.

One method of preparing the water soluble salt of 1-pimamic acid-maleic anhydride adduct which may be either an alkali metal salt, an ammonium salt, or an amine salt, is as follows, illustrating the preparation of the sodium salt: 98 parts of sodium hydroxide pellets were dissolved in 1000 parts of distilled water and the solution was heated on a steam bath with stirring. When the temperature of the solution was about 80° C., 325 parts of 1-pimamic acid-maleic anhydride adduct which had been previously ground to a fine powder were added. Almost immediate solution occurred to produce a dark brown fluid containing 30.2 per cent of solids. This solution was cooled to room temperature, and diluted to the desired concentration and employed for addition to a pulp suspension. The 1-pimamic acid-maleic anhydride adduct is conveniently prepared by heating together 1-pimamic acid and maleic anhydride. A glassy product is obtained thereby, which is ground to a fine powder and used in that form.

If the ammonium salt of the adduct is desired, it may be prepared as follows: 302 parts of commercial grade abietic acid were ground to a fine powder and slowly heated to 210° C. with 98 parts of maleic anhydride. When the temperature had reached 100° C., the mass melted. At 160° C. it began to darken slightly, but the temperature was slowly raised to 210° C. over the period of an hour. After cooling, 100 parts of the finely divided product was added to a mixture of 300 parts of distilled water and 54 parts of 28 per cent aqueous ammonium hydroxide. The resulting clear brown solution was heated briefly with stirring on the steam bath and was diluted with distilled water to a solution having a solids content of 5 per cent.

After the sizing aid has been added to the pulp suspension, there is then added thereto a polyalkyl acrylate resin in the form of its hydrosol, an aqueous dispersion of wax in water and an acid form of aluminum.

The polyalkyl acrylate hydrosol may be prepared as follows: 0.0125 part of potassium persulfate and 1.25 parts of sodium lauryl sulfate were dissolved in 500 parts of distilled water and heated with stirring on a steam bath in a vessel equipped with a reflux condenser, stirrer, and dropping funnel. When the solution had become hot, 125 parts of freshly distilled methyl acrylate was added dropwise with stirring. The polymerization was complete in about 45 minutes. The resultant hydrosol was used in the examples described herein.

The wax dispersion, as employed in accordance with our invention, may be prepared by incorporating a dispersing agent such as glycerol monostearate or some wetting agent in water, and heating the mass on the steam bath to a temperature approaching the boiling point of water. Wax is then added while maintaining the high temperature and the mass is steamed. The elevated temperature melts the wax and it becomes uniformly dispersed in the water. Upon cooling, an aqueous wax dispersion is obtained suitable for use in accordance with our invention. Although paraffin wax has proved to be satisfactory, and because of its price would preferably be employed in actual operations, nevertheless if it is desired, other waxes may be employed, such as

beeswax, carnauba wax, or spermaceti, in preparing the wax dispersion referred to.

The acidic aluminum salt which may be employed is any water soluble salt of aluminum with a strong acid. Aluminum sulfate or aluminum chloride ordinarily comes into use in this connection and either of these salts is suitable for the purpose at hand.

In ordinary operations, our invention is carried out by first subjecting the aqueous slurry of pulp in the beater to a beating operation to obtain the desired slowness—preferably a slowness of 10–50 seconds (Williams). Excessive beating reduces the sizing values and wet strength of the paper prepared therefrom. There is then added the sizing aid, followed by the addition of the hydrosol of the polyalkyl acrylate, the wax dispersion, and the aluminum salt. For best results the aluminum salt should not be contacted with either the resin or the wax dispersion alone, the aluminum salt being the agent which promotes the proper reaction in the pulp suspension. Therefore, for convenience in operation, it is desirable that the aluminum salt be added last.

In preparing the hydrosol of the polyalkyl acrylates, we have found that the surface-active agent which is employed in that preparation should be of anionic type and that it should be not more than 2 per cent and preferably 1 per cent or less (but at least 0.1%) based on the monomer content of the mass. Some surface-active agents which may be employed are sodium higher alcohol sulfates, sodium salts of higher fatty acids, sulfated fatty alcohols, and the like. The alkyl acrylates employed may be either the lower alkyl acrylates of simple acrylic acid such as methyl acrylate or ethyl acrylate or the lower alkyl esters of the methacrylic acids such as methyl methacrylate or ethyl methacrylate.

In carrying out our invention, it is desirable to use an amount of sizing aid, i. e. gelatin or the water soluble salt of pimamic acid-maleic anhydride adduct, abietic acid, or hydrogenated abietic acid, in the proportion of approximately 0.15–1.5%, based on the dry weight of the cellulose pulp which was employed in preparing the paper. The polyalkyl acrylate should be employed to impart the desired properties in an amount such that the proportion thereof is 7.5–15%, based on the dry weight of the pulp employed in making the paper. The wax employed should be in the proportion of 7.5–7.5%, based on the dry weight of the pulp employed in preparing the paper. The aluminum salt of a strong mineral acid which is employed should be added in the proportion of 1–10% based on the dry weight of the pulp which is employed in making the paper.

The following examples illustrate our invention:

*Example 1.*—To 3,000 parts of a 2 1/4 per cent aqueous slurry of an alpha cellulose pulp beaten to a Williams slowness of 20–25 seconds was added the following materials in the order listed:

5 parts of an aqueous solution containing 4.4 per cent of gelatin, 0.12 per cent of formaldehyde, and .007 per cent of chromic chloride deca hydrate

10 parts of a hydrosol of polymethyl acrylate prepared as described above

20 parts of a 10 per cent dispersion of paraffin wax in water using glycerol monostearate as the dispersing agent

25 parts of a 14 per cent aqueous solution of aluminum chloride.

The pulp was then diluted and sheets were formed in a Noble and Wood hand sheet device. The resulting paper was dried for three minutes at 200–210° F. on a rotary drum dryer.

The sheets were tested and the following values were found:

Wet strength, 7 1/4

Cobb size, 0.168

Valley penetration, 24.

The wet strength of the sheets was determined by immersing the sheet for two hours in distilled water at room temperature and then measuring the bursting strength on the Minden paper tester in p. s. i.

5 The Cobb size test is recorded in grams increase in weight, and was measured according to TAPPI standard No. T441 m 45.

10 The Valley penetration recorded in seconds was measured as follows: A 2-inch square sample of paper was mounted between two wooden blocks that had been drilled to allow an electrolyte (516 ml. distilled water, 24 grams of NaCl, 60 ml. glycerine) to contact both sides of the paper simultaneously over a circular area of approximately 1 inch diameter. A potential is applied that allows 200 m. a. of current to flow when no paper sample is present. When a paper sample is mounted in the blocks, the time in seconds is noted from the moment the electrolyte is first brought in contact with the paper sample until 160 m. a. of current flows through the paper sample.

15 *Example 2.*—The procedure of Example 1 was followed exactly except that 50 parts instead of 20 parts of the paraffin wax dispersion was used. Upon testing, the results obtained were as follows:

20 Wet strength, 5 1/2

Cobb size, 0.117

Valley penetration, 55.

25 *Example 3.*—3,000 parts of 2 1/4 percent pulp suspension was beaten to a slowness of 20–25 seconds and there was then added thereto the following materials in the order listed:

30 5 parts of a 5 per cent solution of the sodium salt of 1-pimamic acid-maleic anhydride adduct

35 10 parts of a hydrosol of polyethyl acrylate prepared in the same manner as described above except that ethyl acrylate rather than methyl acrylate was used

40 30 parts of a 10 per cent dispersion of paraffin wax in water using glycerol monostearate as the dispersing agent

45 25 parts of a 14 per cent aqueous solution of aluminum chloride.

The pulp was diluted, sheets were formed therefrom, and the paper was dried as in Example 1. The sheets were tested and gave the following values:

50 Wet strength, 7 1/2

Cobb size, 0.179

Valley penetration, 26.

55 *Example 4.*—3,000 parts of a 2 1/4 percent aqueous slurry of pulp was beaten to a Williams slowness of 20–25 seconds and the following materials in the order listed were added:

60 5 parts of an aqueous solution containing 4.4 per cent of gelatin, 0.12 per cent of formaldehyde, and 0.007 per cent of chromic chloride deca hydrate

65 20 parts of the hydrosol polyethyl acrylate such as described in the preceding example

60 20 parts of a 10 per cent aqueous dispersion of paraffin wax

25 parts of a 14 per cent solution of aluminum chloride in water.

70 The results obtained were as follows:

Wet strength, 7 3/4

Cobb size, 0.181

Valley penetration, 22.

75 We have found that without the use of the combination of the wax dispersion and the polyalkyl acrylate, both high wet strength and resistance to penetration by water are not obtained. Also, the addition of the sizing aid is necessary to assure adherence of the sizing material to the cellulose fibers, while the presence of the aluminum salt is necessary to assure satisfactory sizing operations.

The paper to which high wet strength is imparted by our invention may be any type of paper-making pulp, such as sulfite pulp, kraft pulp, or any other type of pulp which is employed in making paper. We have found that our invention is eminently suitable for use in preparing paper from kraft pulp, both of the bleached and non-bleached type. However, with non-bleached kraft pulp, wet strength and sizing values are obtained which appear to be superior to those of any papers which have been prepared heretofore to our knowledge.

We claim:

1. A high wet strength paper containing therein, based on the dry weight of the pulp employed in its preparation, the following in the proportions given:

|                                                                                                                                                                                                                         | Per Cent |
|-------------------------------------------------------------------------------------------------------------------------------------------------------------------------------------------------------------------------|----------|
| A sizing aid selected from the group consisting of gelatin, water soluble salt of pimamic acid-maleic anhydride adduct, the water soluble salt of abietic acid, and the water soluble salt of hydrogenated abietic acid | 0.15-1.5 |
| Polyalkyl acrylate, the alkyl being of not more than two carbon atoms                                                                                                                                                   | .75-15   |
| Wax                                                                                                                                                                                                                     | .75-7.5  |
| Aluminum salt selected from the group consisting of aluminum sulfate and aluminum chloride                                                                                                                              | 1-10     |

2. A high wet strength paper containing therein, based on the dry weight of the pulp employed in its preparation, the following in the proportions given:

|                                                                                            | Per Cent |
|--------------------------------------------------------------------------------------------|----------|
| Gelatin                                                                                    | 0.15-1.5 |
| Polyalkyl acrylate, the alkyl being of not more than two carbon atoms                      | .75-15   |
| Wax                                                                                        | .75-7.5  |
| Aluminum salt selected from the group consisting of aluminum sulfate and aluminum chloride | 1-10     |

3. A high wet strength paper containing therein, based on the dry weight of the pulp employed in its preparation, the following in the proportions given:

|                                                                                            | Per Cent |
|--------------------------------------------------------------------------------------------|----------|
| A water soluble salt of pimamic acid-maleic anhydride adduct                               | 0.15-1.5 |
| Polyalkyl acrylate, the alkyl being of not more than two carbon atoms                      | .75-15   |
| Wax                                                                                        | .75-7.5  |
| Aluminum salt selected from the group consisting of aluminum sulfate and aluminum chloride | 1-10     |

4. A high wet strength paper containing therein, based on the dry weight of the pulp employed in its preparation, the following in the proportions given:

|         | Per Cent |
|---------|----------|
| Gelatin | 0.15-1.5 |

|                                                                                            | Per Cent |
|--------------------------------------------------------------------------------------------|----------|
| Polymethyl acrylate                                                                        | .75-15   |
| Wax                                                                                        | .75-7.5  |
| Aluminum salt selected from the group consisting of aluminum sulfate and aluminum chloride | 1-10     |

5. A high wet strength paper containing therein, based on the dry weight of the pulp employed in its preparation, the following in the proportions given:

|                                                                                            | Per Cent |
|--------------------------------------------------------------------------------------------|----------|
| A water soluble salt of pimamic acid-maleic anhydride adduct                               | 0.15-1.5 |
| Polymethyl acrylate                                                                        | .75-15   |
| Wax                                                                                        | .75-7.5  |
| Aluminum salt selected from the group consisting of aluminum sulfate and aluminum chloride | 1-10     |

6. A method of preparing high wet strength paper which comprises incorporating into a suspension of paper pulp a sizing aid selected from the group consisting of gelatin, the water soluble salt of pimamic acid-maleic anhydride adduct, the water soluble salt of abietic acid, and the water soluble salt of hydrogenated abietic acid, and then adding thereto a polyalkyl acrylate hydrosol, a wax dispersion, and an aluminum salt selected from the group consisting of aluminum sulfate and aluminum chloride, and then forming paper therefrom.

7. A method of preparing high wet strength paper which comprises incorporating into a suspension of paper pulp a solution of a sodium salt of pimamic acid-maleic anhydride adduct, then adding thereto a polyalkyl acrylate hydrosol, an aqueous dispersion of wax, and an aluminum salt selected from the group consisting of aluminum sulfate and aluminum chloride, and then converting the pulp into paper.

8. A method of preparing high wet strength paper which comprises incorporating into a suspension of paper pulp an aqueous solution of gelatin, then adding thereto a hydrosol of polymethyl acrylate, a dispersion of paraffin wax in water, and an aqueous solution of aluminum chloride, and then forming the pulp into paper.

#### References Cited in the file of this patent

##### UNITED STATES PATENTS

|           |            |       |               |
|-----------|------------|-------|---------------|
| 1,706,841 | Clapp      | ----- | Mar. 26, 1929 |
| 1,942,438 | Manson     | ----- | Jan. 9, 1934  |
| 2,021,172 | Bucy       | ----- | Nov. 19, 1935 |
| 2,119,509 | Barnhart   | ----- | June 7, 1938  |
| 2,315,675 | Trommsdorf | ----- | Apr. 6, 1943  |
| 2,325,302 | Britt      | ----- | July 27, 1943 |
| 2,343,065 | Kumler     | ----- | Feb. 29, 1944 |
| 2,343,090 | Smith      | ----- | Feb. 29, 1944 |
| 2,354,574 | Carson     | ----- | July 25, 1944 |
| 2,539,183 | Child      | ----- | Jan. 23, 1951 |